

March 28, 1950

C. E. LIBBY

2,502,330

WASHING PAPER PULP TO REMOVE COLORING MATTER

Filed March 1, 1943

5 Sheets-Sheet 1

Fig. 1.

THE EFFECT OF DETERGENT WASHING BEFORE EXPOSURE  
TO AIR ON THE BLEACHABILITY OF SULPHATE PULP



INVENTOR

Clarence E. Libby

by

Stibbs, Bleeker & Paruska.  
His Atty.

March 28, 1950

C. E. LIBBY

2,502,330

WASHING PAPER PULP TO REMOVE COLORING MATTER

Filed March 1, 1943

5 Sheets-Sheet 2

Fig. 2.

BURSTING STRENGTH OF BLEACHED SULPHATE PULPS



INVENTOR

Clarence E. Libby

by

Stibbs, Blawie & Parachuk.  
H. J. Stibbs.

March 28, 1950

C. E. LIBBY

2,502,330

WASHING PAPER PULP TO REMOVE COLORING MATTER

Filed March 1, 1943

5 Sheets-Sheet 3

*Fig. 3.*



INVENTOR

Clarence E. Libby  
by  
Stebbins and Blenko.  
His Atty's

March 28, 1950

C. E. LIBBY

2,502,330

WASHING PAPER PULP TO REMOVE COLORING MATTER

Filed March 1, 1943

5 Sheets-Sheet 4

*Fig. 4.*

*BEATER STRENGTH CHARACTERISTICS  
BURST AND TEAR FACTORS*



INVENTOR

Clarence E. Libby

Stebbins and Libby.  
His Atty.

March 28, 1950

C. E. LIBBY

2,502,330

WASHING PAPER PULP TO REMOVE COLORING MATTER

Filed March 1, 1943

5 Sheets-Sheet 5

*Fig. 5.*  
BEATER STRENGTH CHARACTERISTICS OF THE SULFITE PULPS  
BURST FACTOR



Clarence E. Libby  
by  
Stearns and Blake.  
His Atty.

## UNITED STATES PATENT OFFICE

2,502,330

WASHING PAPER PULP TO REMOVE  
COLORING MATTER

Clarence E. Libby, Syracuse, N. Y.

Application March 1, 1943, Serial No. 477,514

8 Claims. (Cl. 92—13)

1

This invention relates to a process of removing coloring matter from paper pulp by any of the commonly used pulping processes, such, for example, as the sulphate (Kraft), soda or sulphite process.

This application is a continuation-in-part of my application, Serial No. 334,178, filed May 8, 1940, now abandoned.

The invention will be described first as applied more particularly to the removal of coloring matter from sulphate pulp. In carrying out the sulphate or Kraft process for producing paper pulp, the chips of wood are digested under pressure with a liquor containing sodium hydroxide and sodium sulphide as the principal constituents and also containing smaller amounts of other materials including sodium carbonate, sodium sulphate, sodium sulphite and sodium thiosulphate. During the digestion or cooking process, the color bodies are to a considerable extent dissolved in the cooking liquor. Unless this liquor is removed from the exterior and interior of the fibers of cellulose at the end of the cook, enough of the color bodies remain on and in the fibers to impart a dark brown color to the paper made from them. These color bodies are organic compounds, either present originally in the wood or derived from reaction of the bodies in the wood with the treating chemicals and are in the nature of tannin or lignin compounds. The constituents of water may contribute to the production of color bodies, either directly or in combination with inorganic compounds. For example, dissolved iron or manganese will be oxidized and precipitated respectively as red hydrous ferric oxide and black manganese hydroxide, or may combine with the organic bodies to produce objectionable color.

Fig. 1 is a graph showing the reflectance values and chlorine consumed in bleaching pulps which had been previously washed with different chemicals while still in the digester and without access of air;

Fig. 2 is a graph showing the bursting strength of bleached sulphate pulps which had been pre-

2

viously washed with different chemicals while in the digester and without access of air.

Fig. 3 is a graph showing the reflectance values and chlorine consumed in bleaching pulps which had been previously washed outside of the digester in the presence of air.

Fig. 4 is a graph showing the beater strength characteristics (burst and tear factors) of the sulphate pulp prepared according to Example 1.

10 Fig. 5 is a graph showing the burst factor of sulphite pulps which were washed prior to bleaching with water or with sodium hexametaphosphate solution.

I have found that the color of the pulp may be 15 materially improved, if it is washed after the digestion step, but before bleaching, with an aqueous solution containing a molecularly dehydrated alkali-metal phosphate. The washing process may be carried out in the digester without allowing access of air to the pulp; or it may be carried 20 out in the presence of air, for example, in washing pits or upon continuous rotary filters.

The preferred molecularly dehydrated alkali-metal phosphate is the glassy phosphate commonly known as Graham's salt or sodium hexametaphosphate, which has a mol ratio of  $Na_2O$  to  $P_2O_5$  of 1:1. It will be understood that this

25 sodium phosphate glass is given as representative of the family of glassy molecularly dehydrated phosphates and that other glassy molecularly dehydrated phosphates having a mol ratio of  $Na_2O$  to  $P_2O_5$  between 0.9:1.0 and 1.7:1.0, such as the so-called sodium tetraphosphate  $Na_6P_4O_{13}$ , with a mol ratio of  $Na_2O$  to  $P_2O_5$  of 1.5:1.0 or the

30 so-called sodium decaphosphate,  $Na_{12}P_{10}O_{31}$ , with a mol ratio of  $Na_2O$  to  $P_2O_5$  of 1.2:1.0, may be used in place of or in addition to sodium hexametaphosphate. All of these glassy phosphates have properties which are similar to one another,

35 although differing somewhat in their effectiveness.

I may use in place of or in addition to the glassy molecularly dehydrated alkali-metal phosphates the alkali-metal tripolyphosphates, for 40 example, sodium tripolyphosphate,  $Na_5P_3O_{10}$ , or

the alkali-metal pyrophosphates, for example, tetrasodium pyrophosphate,  $Na_4P_2O_7$ .

The common practice in counteracting the bad effects of the color bodies in paper pulp is to wash the pulp with water or with weak black liquor followed by water and then to bleach the pulp. I have found that greatly superior results are obtained by washing the pulp with water containing molecularly dehydrated alkali-metal phosphates, as compared with the results obtained in using the commonly known washing methods. I also have found that the molecularly dehydrated alkali-metal phosphates produce materially superior results as compared with the use of caustic soda or other ordinary detergents. These superior results are shown by the lower chlorine demand in bleaching the pulp, the higher reflectance of the bleached pulp and the higher retention of strength in the bleached pulp.

Figs. 1 and 2 show the results obtained by washing a sulphate pulp after digestion but before contact with air with water alone or with aqueous solutions containing various chemicals. The washed pulp was then bleached with a chlorine bleaching agent and reflectance values and bursting strength values for the different samples were obtained. The bleached pulp which had been washed with sodium hexametaphosphate solution attained higher reflectance values than the pulp washed with any of the other chemicals.

In carrying out the washing process, the pulp was treated in the digester after the digestion step had been completed. The cooking liquor was drained from the digester and a washing solution was circulated through the digester while excluding air. The circulation of the washing solution was continued for approximately thirty minutes per wash and the washing liquors were maintained at about  $100^{\circ} C$ . Table I lists the compounds which were investigated, the ratio by weight of compound to wood, and the number and length of the washes.

TABLE II  
BLEACHABILITY TESTS OF WASHED KRAFT PULPS

| 5  | Cook No. | Percent Cl Added | Percent Cl Consumed | Higgins Reflectance | Natural Cl Consumption |
|----|----------|------------------|---------------------|---------------------|------------------------|
| 10 | 1.....   | 7                | 6.93                | 57                  |                        |
|    | 1.....   | 9                | 8.54                | 58.3                |                        |
|    | 1.....   | 11               | 10.18               | 60                  |                        |
|    | 1.....   | 13               | 11.72               | 65.5                |                        |
|    | 1.....   | 15               | 13.16               | 69                  |                        |
|    | 2.....   | 7                | 6.53                | 61.5                |                        |
|    | 2.....   | 9                | 7.86                | 63                  |                        |
|    | 2.....   | 11               | 9.34                | 64                  | 11.5                   |
|    | 2.....   | 13               | 11.52               | 71                  |                        |
|    | 2.....   | 15               | 13.19               | 71                  |                        |
| 15 | 3.....   | 7                | 6.47                | 66                  |                        |
|    | 3.....   | 9                | 7.67                | 67                  |                        |
|    | 3.....   | 11               | 9.41                | 68.5                | 11.0                   |
|    | 3.....   | 13               | 11.49               | 72                  |                        |
|    | 3.....   | 15               | 13.22               | 73                  |                        |
|    | 4.....   | 7                | 6.80                | 62.5                |                        |
|    | 4.....   | 9                | 8.06                | 68                  |                        |
|    | 4.....   | 11               | 9.95                | 77.8                | 10.0                   |
|    | 4.....   | 13               | 11.89               | 75                  |                        |
|    | 4.....   | 15               | 13.73               | 77                  |                        |
| 20 | 5.....   | 7                | 6.89                | 58                  |                        |
|    | 5.....   | 9                | 8.49                | 65                  |                        |
|    | 5.....   | 11               | 10.38               | 77                  |                        |
|    | 5.....   | 13               | 12.13               | 73.5                |                        |
|    | 5.....   | 15               | 14.08               | 74                  |                        |
|    | 6.....   | 7                | 7.00                | 36                  |                        |
|    | 6.....   | 9                | 8.92                | 52.5                |                        |
|    | 6.....   | 11               | 10.93               | 61.5                | 12.25                  |
|    | 6.....   | 13               | 12.75               | 62.5                |                        |
|    | 6.....   | 15               | 14.52               | 68                  |                        |
| 25 | 7.....   | 7                | 7.00                | 39                  |                        |
|    | 7.....   | 9                | 9.00                | 49                  |                        |
|    | 7.....   | 11               | 10.94               | 60                  |                        |
|    | 7.....   | 13               | 12.67               | 65                  |                        |
|    | 7.....   | 15               | 14.16               | 62.8                |                        |
|    | 7.....   | 7                | 6.78                | 62                  |                        |
|    | 8.....   | 9                | 7.94                | 67                  |                        |
|    | 8.....   | 11               | 9.98                | 78.5                | 10.00                  |
|    | 8.....   | 13               | 11.76               | 76.8                |                        |
|    | 8.....   | 15               | 13.08               | 75.5                |                        |
| 30 | 9.....   | 7                | 6.93                | 57                  |                        |
|    | 9.....   | 9                | 8.89                | 64                  |                        |
|    | 9.....   | 11               | 10.60               | 69                  |                        |
|    | 9.....   | 13               | 12.26               | 70                  |                        |
|    | 9.....   | 15               | 13.78               | 72                  |                        |
|    | 9.....   | 7                | 6.81                | 62.5                |                        |
|    | 10.....  | 9                | 8.11                | 68.5                |                        |
|    | 10.....  | 11               | 8.97                | 72.5                |                        |
|    | 10.....  | 13               | 9.09                | 71                  |                        |
|    | 10.....  | 15               | 10.74               | 72                  |                        |

It should be noted that while all pulps are difficult to bleach, requiring from 9 to 12.5% of

TABLE I

## DETERGENT WASHING OF KRAFT PULP

| Cook No. | Washing Agent                  | Grams per Wash | Schedule                 | Compound on Oven Dry Chips |
|----------|--------------------------------|----------------|--------------------------|----------------------------|
| 1.....   | Water.....                     |                | Continuous 30 lb. press. | Per cent                   |
| 2.....   | $Na_2O \cdot 3.22 SiO_2$ ..... | 150            | 1 wash, 30 min.....      | 5                          |
| 3.....   | do.....                        | 150            | 2 washes, 30 min. each.  | 10                         |
| 4.....   | Sodium Hexametaphosphate.....  | 150            | 1 wash, 30 min.....      | 5                          |
| 5.....   | $Na_2S$ .....                  | 150            | 1 wash, 30 min.....      | 5                          |
| 6.....   | $NaOH$ .....                   | 150            | 1 wash, 30 min.....      | 6                          |
| 7.....   | Red Oil Soap.....              | 150            | 1 wash, 30 min.....      | 5                          |
| 8.....   | Sodium Hexametaphosphate.....  | 150            | 1 wash, 30 min.....      | 5                          |
| 9.....   | Red Oil Soap.....              | 30             | 1 wash, 30 min.....      | 5                          |
| 10.....  | $Na_4P_2O_7$ .....             | 75             | 2 washes, 30 min. each.  | 5                          |
| 10.....  | $Na_2S_2O_4$ .....             | 75             | 2 washes, 30 min. each.  | 5                          |

After the washing had been completed, the pulps were bleached using calcium hypochlorite bleaching liquor and the bleached pulp samples were made into sheets and tested for brightness by the Higgins color analyzer. Table II is a tabulation of the bleaching data both as to quantity of chlorine added and consumed and the results obtained in terms of brightness of the finished pulps.

chlorine, the results are strictly comparable and actually duplicate some commercial pulps which are cooked primarily for strength and not for a high white color on bleaching.

Fig. 1 presents graphically the data tabulated in Table II.

The effect of washing with different chemicals before exposure to air on the bleachability of sulphate pulp is shown in Fig. 1, which gives the

Higgins reflectance values and the per cent chlorine consumed in bleaching the different samples which had been previously washed in digester without access of air with aqueous solutions of the different chemicals given in Table I. It will be seen from this figure and from Table II that sodium hexametaphosphate (curve 4) and sodium hexametaphosphate plus soap (curve 8) when used as washing solutions gave higher reflectance values of the bleached pulp than any of the other chemicals.

The following tests were made on the pulps before and after bleaching:

Beater strength tests were made according to T. A. P. P. I. standard T-200 M-40.

Bursting strength tests were made according to T. A. P. P. I. standard T-403 M-36.

Tearing strength tests were made according to T. A. P. P. I. standard T-414 M-40.

Bleachability was determined by a single-stage hypochlorite bleach commonly known as the "Excess chemical method." The bleachability as recorded in the tables refers to the per cent of chlorine on the weight of oven-dry pulp that is required to give an 80% brightness reading on the Higgins photoelectric colorimeter.

Pulps washed with metaphosphate show higher physical properties than those washed with other chemicals. The most common test employed for the evaluation of pulps is the beating strength test in which a weighed quantity of pulp, e. g. 500 grams, is beaten in a small strength testing beater for a period of time or until the maximum bursting strength of the pulp has been developed. All pulps increase in strength as the beating progresses until a maximum is reached, after which the bursting strength decreases in value. As the strength increases the freeness, as measured by the amount of water which will drain from a weighed quantity of the pulp suspended in 1000 cubic centimeters of water in the standard freeness testing instrument, rapidly decreases. It is customary to beat pulps until the freeness decreases to 50 ml., at which time the maximum strength will have been passed in almost all cases. The bursting strength is determined by making sheets of the beating pulp on a standard sheet mould, drying at a given temperature, conditioning the dried sheets in an atmosphere of 65% relative humidity and 70° F. for a period of 10 hours and then testing on a Mullen bursting strength tester. This instrument consists of a chamber filled with glycerine into which a plunger is forced at a constant rate, this action forcing the glycerine against a rubber diaphragm over which the sample sheet is clamped. The rubber diaphragm has an area of one square inch so that the results are recorded in terms of pounds per square inch required to burst the sample, the instrument having a pressure gauge attached to the glycerine chamber. The sample sheets are usually made to some standard weight basis, e. g. 50 pounds per ream, 25 x 40—500. Since unavoidable variations in basis weight will occur, it is customary to divide the bursting strength test value by the basis weight of the sheet being tested, the result being reported as "burst factor." A similar report is made for all other physical tests. This form of report compensates for irregular results, due to variations in the thickness and weight of the test sheets.

It should be noted that the "burst factor" is considered the most important criterion of the quality of a pulp. Many mills make no other test, although some use a Tear test which always

progressively decreases as beating progresses, due to shortening of the pulp fibers. When the "burst factor" of a paper equals 1.0 points, known to mill operators as "point to a pound," the pulp is considered highly satisfactory, especially if the pulp has been bleached.

Table III is a tabulation of the strength data obtained by a series of physical tests on the Kraft pulps which has been washed before bleaching with various detergent compounds.

TABLE III  
STRENGTH EVALUATION OF DETERGENT WASHED  
KRAFT PULPS

|                | Washing Agent                                | Beating Time Minutes           | Canadian Standard Freeness | Burst Factor      | Tear Factor          | Bulk Factor          |
|----------------|----------------------------------------------|--------------------------------|----------------------------|-------------------|----------------------|----------------------|
| 15             | H <sub>2</sub> O Wash<br>Unbleached<br>#1    | 5                              | 720                        | .71               | 3.93                 | 2.57                 |
|                |                                              | 20                             | 350                        | 1.07              | 2.75                 | 1.56                 |
|                |                                              | 35                             | 130                        | 1.03              | 2.78                 | 1.81                 |
|                |                                              | 50                             | 25                         | 1.49              | 2.28                 | 1.74                 |
| BLEACHED PULPS |                                              |                                |                            |                   |                      |                      |
| 25             | H <sub>2</sub> O Wash<br>#1                  | 5                              | 680                        | .71               | 1.87                 | 1.85                 |
|                |                                              | 20                             | 190                        | .73               | 1.80                 | 1.48                 |
|                |                                              | 35                             | 27                         | .70               | 1.30                 | 1.25                 |
|                |                                              | Sodium Silicate<br>#2          | 560<br>125<br>38           | .53<br>.53<br>.57 | 1.16<br>1.04<br>.78  | 1.73<br>1.66<br>1.70 |
| 30             | Sodium Silicate<br>#3                        | 5                              | 575                        | .69               | 1.68                 | 1.73                 |
|                |                                              | 20                             | 102                        | .63               | .97                  | 1.31                 |
|                |                                              | 24                             | 58                         | .64               | .80                  | 1.17                 |
|                |                                              | Sodium Hexametaphosphate<br>#4 | 580<br>104<br>50           | .89<br>.89<br>.98 | 1.72<br>1.10<br>1.15 | 1.65<br>1.49<br>1.32 |
| 35             | Sodium Sulfide<br>#5                         | 5                              | 680                        | .57               | 1.62                 | 1.76                 |
|                |                                              | 20                             | 360                        | .80               | 1.22                 | 1.53                 |
|                |                                              | 35                             | 85                         | .84               | 1.10                 | 1.29                 |
|                |                                              | 38                             | 56                         | .77               | .95                  | 1.21                 |
| 40             | Sodium Hydroxide<br>#6                       | 5                              | 690                        | .64               | 1.68                 | 1.82                 |
|                |                                              | 20                             | 365                        | .88               | 1.28                 | 1.60                 |
|                |                                              | 35                             | 110                        | .98               | 1.16                 | 1.18                 |
|                |                                              | 40                             | 50                         | .87               | 1.06                 | 1.09                 |
| 45             | Sodium Oleate<br>#7                          | 5                              | 730                        | .63               | 1.70                 | 1.69                 |
|                |                                              | 20                             | 425                        | .76               | 1.38                 | 1.51                 |
|                |                                              | 35                             | 140                        | .91               | 1.18                 | 1.34                 |
|                |                                              | 43                             | 58                         | .70               | 1.12                 | 1.24                 |
| 50             | Soap 1%<br>Sodium Hexametaphosphate<br>5%—#8 | 5                              | 690                        | .65               | 1.74                 | 1.63                 |
|                |                                              | 20                             | 425                        | .90               | 1.38                 | 1.39                 |
|                |                                              | 35                             | 160                        | .90               | 1.37                 | 1.16                 |
|                |                                              | 44                             | 59                         | 1.04              | 1.05                 | 1.02                 |
| 55             | Tetra Sodium Pyrophosphate<br>#9             | 5                              | 700                        | .61               | 1.38                 | 1.74                 |
|                |                                              | 20                             | 320                        | .77               | 1.13                 | 1.48                 |
|                |                                              | 35                             | 63                         | .71               | .89                  | 1.26                 |
|                |                                              | 37                             | 47                         | .79               | .87                  | 1.17                 |
| 60             | Sodium Hydrogen Sulfite<br>#10               | 5                              | 700                        | .65               | 1.54                 | 1.67                 |
|                |                                              | 20                             | 350                        | .89               | 1.12                 | 1.41                 |
|                |                                              | 35                             | 73                         | .81               | .86                  | 1.13                 |
|                |                                              | 38                             | 47                         | .73               | .99                  | 1.14                 |

An examination of the data in Table III shows that the only bleached pulps which even closely approached the ideal strength of a "point to a pound" were the products of Runs Nos. 4 and 8 which had been washed with metaphosphate.

An inspection of the curves of Fig. 2 shows that Runs Nos. 4 and 8 not only have a higher maximum "burst factor" than any of the other pulps but that the strength values shown are not maximum factors, since the strengths are still increasing. This fact may be very important in that it indicates the probability that more fully cooked pulps may be even proportionately stronger when washed with metaphosphate, since drastic bleaching treatment does not appear to be necessary to remove the colored impurities which remain after the metaphosphate treatment.

In the preceding tests, relatively large amounts of metaphosphate were employed in the washing of the pulp. It has been found, however, that

advantageous saving in chlorine and conservation in strength of the pulp may be obtained, even when relatively small amounts of metaphosphate are present in the water used for washing.

The following is an example of one method of treating sulphate pulp according to the present invention:

*Example 1*

Dry wood used \_\_\_\_\_ grams 3000  
 Active chemical as  $\text{Na}_2\text{O}$  \_\_\_\_\_ per cent 20  
 Sulphidity \_\_\_\_\_ do 33 1/3  
 Liquor ratio \_\_\_\_\_ 5 to 1

The volume of black liquor employed was approximately 44% of the total volume of liquor in the digester and contained 7.5% of the total NaOH requirement calculated as  $\text{Na}_2\text{O}$ .

Cooking schedule:

1 1/2 hours to reach maximum temperature of 170° C.

3 hours at maximum temperature.

Method of washing:

1. Weak black liquor at 75° C.—20 minutes.

2. Fresh water + sodium hexametaphosphate at 75° C.—20 minutes.

3. Fresh water + sodium hexametaphosphate at 75° C.—20 minutes.

compared with a maximum burst factor of 1.33 for the bleached pulp washed with water. In other words, the bleached pulp previously washed with sodium hexametaphosphate retains a considerably higher percentage of its unbleached strength as shown by the burst factor than does the bleached pulp previously washed with water.

It can also be seen from Fig. 4 that washing with sodium hexametaphosphate and bleaching produces substantially higher tear factors than washing with water and bleaching of the pulp.

Washing solutions of molecularly dehydrated alkali-metal phosphates may also be employed to remove color in the treatment of soda pulps prior to bleaching. The following is an example:

*Example 2*

These pulps were prepared under the following conditions:

Dry wood used \_\_\_\_\_ grams 3000  
 Active chemical as  $\text{Na}_2\text{O}$  \_\_\_\_\_ per cent 19.5

Liquor ratio \_\_\_\_\_ 6 to 1

Cooking schedule:

1 1/2 hours to reach maximum temperature of 178° C.

2 hours at maximum temperature.

Method of washing:

1. Weak black liquor at 75° C.—20 minutes.

| Cook No. | Per cent Sodium hexametaphosphate used <sup>1</sup> | Un-screened Yield, per cent | Screened Yield, per cent | Screenings, per cent | Bleachability <sup>2</sup> | Actual overall chlorine consumption in 3 stage bleach <sup>3</sup> |      |       |
|----------|-----------------------------------------------------|-----------------------------|--------------------------|----------------------|----------------------------|--------------------------------------------------------------------|------|-------|
|          |                                                     |                             |                          |                      |                            | 1st                                                                | 3rd  | Total |
| 28       |                                                     | 47.4                        | 44.7                     | .30                  | 12.0                       | 3.86                                                               | 1.71 | 5.57  |
| 27       | 0.02                                                | 47.2                        | 44.8                     | .31                  | 9.4                        | 3.34                                                               | 1.68 | 4.92  |
| 48       | 0.02                                                | 46.8                        | 44.6                     | .35                  | 9.0                        | 3.33                                                               | 1.57 | 4.90  |

<sup>1</sup> Based on weight of wood.

<sup>2</sup> Per cent chlorine to give 80 brightness in single-stage bleach.

<sup>3</sup> The second stage of bleaching consisted of an alkaline extraction using 1% of NaOH on the weight of pulp, conducted at 40° C. for one hour.

NOTE.—Cook 27 was washed inside the digester in the absence of air, cook 48 was washed outside the digester in the presence of air.

*Bleachability Determinations*

|                                                        |                            |      |      |       |       |       |       |    |
|--------------------------------------------------------|----------------------------|------|------|-------|-------|-------|-------|----|
| Cook No. 28 Water Washed                               | Per cent chlorine consumed | 7.0  | 8.81 | 10.49 | 12.31 | 14.16 | 16.09 | 45 |
| Brightness                                             |                            | 64.0 | 75.0 | 78.5  | 80.5  | 81.0  | 81.5  |    |
| Cook No. 27 Washed with 0.02% Sodium Hexametaphosphate | Per cent chlorine consumed | 6.93 | 8.71 | 10.48 | 12.29 | 14.23 | 16.16 |    |
| Brightness                                             |                            | 72.5 | 78.5 | 81.5  | 82.0  | 83.0  | 84.0  |    |
| Cook No. 48 Washed with 0.02% Sodium Hexametaphosphate | Per cent chlorine consumed | 6.98 | 8.85 | 10.07 | 12.56 | 14.55 | 16.83 | 50 |
| Brightness                                             |                            | 72.0 | 79.0 | 81.5  | 82.0  | 83.0  | 83.0  |    |

This example shows a very considerable saving in the chlorine consumption during bleaching as a result of using in the washing operation 0.02% of sodium hexametaphosphate based upon the weight of the wood. In the single-stage measurement of the bleachability, the chlorine consumption to attain a brightness of 80 was reduced from 12.0% for pulp washed with water alone to 9.4 and 9.0 for the pulp washed with sodium hexametaphosphate solution. The overall chlorine consumption in a three-stage bleach corresponding more closely to common plant practice was correspondingly reduced from 5.57% for pulp washed with water alone to 4.92% and 4.90% for pulp washed with water containing 0.02% of sodium metaphosphate. The bleachability determinations given in Example 1 for Cooks No. 28 and 48 are shown graphically in Fig. 3.

The beater strength characteristics (burst factor and tear factor) of the sulphate pulp prepared according to Example 1 are shown in Fig. 4. It will be noted from Fig. 4 that the burst factor for the bleached pulp made by washing with sodium hexametaphosphate solution prior to bleaching has a maximum value of about 1.44 as

2. Weaker black liquor at 75° C.—20 minutes.  
 3. Fresh water + sodium hexametaphosphate at 85° C.—20 minutes.

| Cook No. | Per cent Sodium hexametaphosphate <sup>1</sup> | Un-screened Yield, Per cent | Screened Yield, Per cent | Screenings, Per cent | Actual chlorine consumption in single-step hypochlorite bleach <sup>2</sup> |
|----------|------------------------------------------------|-----------------------------|--------------------------|----------------------|-----------------------------------------------------------------------------|
| 37       |                                                | 44.0                        |                          |                      |                                                                             |
| 39       | 0.02                                           | 43.2                        | 41.2                     | 1.76                 | 3.8                                                                         |

Saving in chlorine on single-stage hypochlorite bleach = 12.6%.

<sup>1</sup> Based on dry weight of wood.

<sup>2</sup> To give 65 brightness.

As in the case of sulphate and soda pulps, the invention also is applicable to the treatment of sulphite pulps by the employment of molecularly dehydrated alkali-metal phosphate solutions to remove color from the pulp prior to bleaching in order to decrease the bleaching requirements and improve the strength retention of the pulps. The sulphite pulps were prepared under the following conditions:

*Example 3*

Dry wood used \_\_\_\_\_ 3000 grams  
 Sulphite cooking liquor \_\_\_\_\_ 5.0% Free  $\text{SO}_2$   
 70 1.3% Combined  $\text{SO}_2$   
 6.3% Total  $\text{SO}_2$

Liquor ratio \_\_\_\_\_ 6 to 1  
 Cooking schedule: At the end of 2 hours, the temperature of the cook was 110° C., and at the end of 6 hours it was 140° C. It was maintained

at this temperature for 3 hours and at the end of a total period of 10 hours was 130° C.

These sulphite pulps were washed with cold water or sodium hexametaphosphate solutions. Each cook was given four washes of 18 liters each for a total of 72 liters, equivalent to about 50 pounds of solution to one pound of pulp.

The pulp was removed from the digester and placed in a disintegration tank and agitated for 20 minutes in cold water. The pulp was placed on a flat screen, excess water removed, and the yield determined at this point. The pulp was screened and all tests were carried out on the screened pulp.

From the bleachability determination it was possible to approximate the quantity of chlorine needed to bleach the pulp using the two-stage bleaching procedure. The equivalent of 550 grams of pulp was bleached to a brightness of 80 per cent on the Higgins photo-electric colorimeter. The first stage of the bleaching procedure was the chlorination stage. Chlorine water was added to the pulp which was kept at 25° C. and a final consistency of 3%. At the end of 90 minutes after determining the amount of chlorine actually consumed, the pulp was completely washed with water. The second stage of the bleaching procedure, or hypochlorite stage, was carried out at 35-37° C. and at a consistency of 5%. Calcium hypochlorite was added to the pulp, sample sheets were made at intervals, and when the brightness of the sheets, as determined by the Higgins photo-electric colorimeter, was 80%, the actual consumption of chlorine was measured and the pulp was again washed with water. The pH of this stage was maintained between 8.5 and 8.9. Total chlorine consumed was the sum of the chlorine consumed in both stages.

Freeness was determined by the Canadian standard freeness tester, using a 0.3% consistency at 20° C., and the results recorded in cubic centimeters.

Prior to testing both the bleached and unbleached sheets, the sheets were conditioned in the paper testing laboratory for 16 hours in an atmosphere maintained at 73° F. and 50% relative humidity and all tests were carried out under these conditions.

The results obtained are shown in the following table:

TABLE IV

| Cook No. | Sodium Hexametaphosphate Used |                           | Un-screened Yield, percent | Screened Yield, percent | Screenings, percent | Bleachability <sup>1</sup> | Actual overall chlorine consumption in 2 stage bleach, percent Cl <sub>2</sub> |           |       |
|----------|-------------------------------|---------------------------|----------------------------|-------------------------|---------------------|----------------------------|--------------------------------------------------------------------------------|-----------|-------|
|          | Cone., P. P. M.               | Percent Based on Dry Wood |                            |                         |                     |                            | 1st Stage                                                                      | 2nd Stage | Total |
| 2        | 20                            | .06                       | 48.75                      | 47.22                   | 1.53                | 4.3                        | -----                                                                          | -----     | ----- |
| 4        | 50                            | .12                       | 48.4                       | 46.81                   | 1.59                | 3.7                        | -----                                                                          | -----     | ----- |
| 5        | 50                            | .12                       | 48.7                       | 47.11                   | 1.59                | 5.5                        | 1.46                                                                           | 1.20      | 2.66  |
| 6        | 35                            | .08                       | 48.3                       | 46.79                   | 1.51                | 3.2                        | 1.25                                                                           | .86       | 2.11  |

<sup>1</sup> Percent chlorine to give 80 brightness in single-stage bleach.

The table shows that the chlorine consumption of the pulp washed with sodium hexametaphosphate was considerably less than that of the pulp washed with water. Whereas it required 5.5% of chlorine to give 80 brightness in a single-stage bleach when the pulp was washed with water, it required only 3.2% or 3.7% or 4.3% of chlorine, depending upon the concentration of the sodium hexametaphosphate when the sodium

the amount of the metaphosphate employed. Expressed in another manner, the washing solution should contain at least about 20 parts of sodium hexametaphosphate per million parts of water. As the concentration is increased up to about 100 parts per million, somewhat improved results are obtained; but beyond this an increase in the concentration of metaphosphate is probably not justified, from an economic standpoint.

hexametaphosphate solutions were employed. In the two-stage bleach, the amount of chlorine required was considerably less for the pulp washed with sodium hexametaphosphate than in the case of the water-washed pulp.

Fig. 5 gives the burst factor for bleached and unbleached sulphite pulps prepared according to Example 3, the bleached pulps having been washed with water or with a 35 P. P. M. aqueous solution of sodium hexametaphosphate and thereafter bleached to a brightness of 80. This graph again illustrates the improved strength characteristics of pulp washed with sodium hexametaphosphate prior to bleaching.

Cuprammonium disperse viscosity tests were made according to T. A. P. P. I. standard T-206 M-37.

Cuprammonium disperse viscosity tests of the sulphite pulps are given in the following table in centipoises:

TABLE V

|    |                                                         | Unbleached | Bleached |
|----|---------------------------------------------------------|------------|----------|
| 25 | Cook No. 5 Water Washed.....                            | 85.2       | 41.2     |
|    | Cook No. 6 Sodium Metaphosphate Washed, 35 P. P. M..... | 85.5       | 48.9     |

The viscosity of the bleached pulp previously washed with sodium hexametaphosphate is considerably higher than that of the water-washed bleached pulp, showing that less degradation of the pulp occurred in the case where it was treated with the sodium hexametaphosphate solution.

The temperature at which the washing with the molecularly dehydrated alkali-metal phosphate is carried out is not critical but may be varied over a wide range. Any washing temperatures up to the boiling point of the washing solution might be employed.

In order to produce materially improved results as compared with washing with water, about 0.02% of sodium hexametaphosphate based on the weight of the dry wood should be employed.

As the amount of sodium hexametaphosphate is increased up to about 0.1% based on the weight of the dry wood, the results are improved somewhat; but beyond this concentration, the improvement in results probably is not sufficient, from the standpoint of cost, to justify increasing

The following table illustrates results which have been obtained with regard to bleachability, chlorine consumption and retention of strength, employing different temperatures and quantities of sodium hexametaphosphate, in the washing of various kinds of pulps:

TABLE VI

| Pulping Process | Washing Temperature, °C. | Sodium Hexameta-phosphate in Wash Water <sup>1</sup> | Bleach-ability <sup>2</sup> | Chlorine Consumption, Multi-stage Bleach |                          | Retention of Strength: |
|-----------------|--------------------------|------------------------------------------------------|-----------------------------|------------------------------------------|--------------------------|------------------------|
|                 |                          |                                                      |                             | Stages                                   | Total Chlorine, Per Cent |                        |
| Sulphate....    | 100                      | 0                                                    | 13.8                        | 3                                        | 5.45                     | 85.0                   |
|                 | 100                      | 0.02                                                 | 10.4                        | 3                                        | 4.74                     | 91.0                   |
|                 | 75                       | 0                                                    | 12.0                        | 3                                        | 5.57                     | 87.0                   |
|                 | 75                       | 0.02                                                 | 9.4                         | 3                                        | 4.92                     | 95.5                   |
|                 | 75                       | 0.02                                                 | 9.0                         | 3                                        | 4.90                     | 90.0                   |
|                 | 50                       | 0                                                    | 12.5                        | 3                                        | 5.95                     | 86.5                   |
| Soda.....       | 50                       | 0.02                                                 | 11.2                        | 3                                        | 5.37                     | 94.5                   |
|                 | 75-85                    | 0                                                    | 3.8                         | -----                                    | -----                    | 85.0                   |
|                 | 75-85                    | 0.02                                                 | 3.32                        | -----                                    | -----                    | 91.0                   |
| Sulphite....    | 20                       | 0                                                    | 5.5                         | 2                                        | 2.66                     | 87.0                   |
|                 | 20                       | 0.05                                                 | 4.3                         | -----                                    | -----                    | -----                  |
|                 | 20                       | 0.09                                                 | 3.2                         | 2                                        | 2.11                     | 95.0                   |
|                 | 20                       | 0.12                                                 | 3.7                         | -----                                    | -----                    | -----                  |

<sup>1</sup> Per cent on weight of dry wood.

<sup>2</sup> Per cent chlorine to give 80 brightness in single-stage bleach, except in case of soda pulp, for which brightness of 65 was used.

<sup>3</sup> As measured by burst factor, per cent of unbleached strength.

In washing the digested pulp with the molecularly dehydrated alkali-metal phosphate solution prior to bleaching, the time of washing and other conditions will, of course, be governed by the amount of coloring matter in the pulp and the desired whiteness of the bleached pulp. Multi-stage and countercurrent washing of the pulp are advantageous under many conditions.

The term "molecularly dehydrated alkali-metal phosphate" is intended to include any of the phosphate glasses previously referred to, as well as the alkali-metal tripolyphosphates or pyrophosphates, both of which are crystalline materials, or mixtures of any of these phosphates. All of these molecularly dehydrated phosphates may be considered as derived from orthophosphates by the elimination of water of constitution. The molecularly dehydrated phosphates contain less water of constitution than the corresponding orthophosphates and have, therefore, come to be recognized as molecularly dehydrated phosphates, as pointed out more fully in the Hall and Jackson Patent 1,903,041, granted March 28, 1933.

Although I have given specific examples and preferred embodiments of the invention, it will be understood that it is not limited thereto but may be otherwise embodied or practiced within the scope of the following claims:

I claim:

1. In the process of removing organic coloring matter in the nature of tannin or lignin compounds from paper pulp without removing a substantial amount of cellulose constituent of the pulp, the step comprising washing the pulp after digestion but before bleaching with a solution consisting essentially of water and about 20 to 100 parts of molecularly dehydrated alkali metal phosphate per one million parts of water, the concentration of molecularly dehydrated alkali metal phosphate in the wash water being substantially less than that which would be required to soften the water by sequestration of calcium.

2. In the process of removing organic coloring matter in the nature of tannin or lignin compounds from paper pulp without removing a sub-

stantial amount of cellulose constituent of the pulp, the step comprising washing the pulp after digestion but before bleaching with a solution consisting essentially of water and about 20 to 100 parts of glassy molecularly dehydrated phosphate having a molecular ratio of Na<sub>2</sub>O to P<sub>2</sub>O<sub>5</sub>

30 between 0.9:1 and 1.7:1 per one million parts of water, the concentration of molecularly dehydrated phosphate in the wash water being substantially less than that which would be required to soften the water by sequestration of calcium.

35 3. In the process of removing organic coloring matter in the nature of tannin or lignin compounds from paper pulp without removing a substantial amount of cellulose constituent of the pulp, the step comprising washing the pulp after digestion but before bleaching with a solution consisting essentially of water and about 20 to 100 parts of Graham's salt per million parts of water, the concentration of Graham's salt in the wash water being substantially less than that which would be required to soften the water by sequestration of calcium.

40 4. In the process of removing organic coloring matter in the nature of tannin or lignin compounds from paper pulp made by the sulphate process without removing a substantial amount of cellulose constituent of the pulp, the step comprising washing the pulp after digestion but before bleaching with a solution consisting essentially of water and about 20 to 100 parts of molecularly dehydrated alkali metal phosphate per one million parts of water, the concentration of molecularly dehydrated alkali metal phosphate in the wash water being substantially less than that which would be required to soften the water by sequestration of calcium.

45 5. In the process of removing organic coloring matter in the nature of tannin or lignin compounds from paper pulp made by the soda process without removing a substantial amount of cellulose constituent of the pulp, the step comprising washing the pulp after digestion but before bleaching with a solution consisting essentially of water and about 20 to 100 parts of molecularly dehydrated alkali metal phosphate per one million parts of water, the concentration of molecularly dehydrated alkali metal phosphate in the wash water being substantially less than that which would be required to soften the water by sequestration of calcium.

50 6. In the process of removing organic coloring matter in the nature of tannin or lignin com-

pounds from paper pulp made by the sulphite process without removing a substantial amount of cellulose constituent of the pulp, the step comprising washing the pulp after digestion but before bleaching with a solution consisting essentially of water and about 20 to 100 parts of molecularly dehydrated alkali metal phosphate per one million parts of water, the concentration of molecularly dehydrated alkali metal phosphate in the wash water being substantially less than that which would be required to soften the water by sequestration of calcium.

7. In the process of removing organic coloring matter in the nature of tannin or lignin compounds from paper pulp without removing a substantial amount of cellulose constituent of the pulp, the step comprising washing the pulp after digestion but before bleaching with a solution consisting essentially of water and about 20 to 100 parts of alkali metal pyrophosphate per one million parts of water, the concentration of alkali metal pyrophosphate in the wash water being substantially less than that which would be required to soften the water by sequestration of calcium.

8. In the process of removing organic coloring matter in the nature of tannin or lignin compounds from paper pulp without removing a substantial amount of cellulose constituent of the pulp, the step comprising washing the pulp after digestion but before bleaching with a solution consisting essentially of water and about 20 to 100 parts of alkali metal tripolyphosphate per one million parts of water, the concentration of alkali metal tripolyphosphate in the wash water being substantially less than that which would be required to soften the water by sequestration of calcium.

CLARENCE E. LIBBY.

REFERENCES CITED

The following references are of record in the file of this patent:

UNITED STATES PATENTS

| Number       | Name     | Date           |
|--------------|----------|----------------|
| 1,435,332    | Phair    | Nov. 14, 1922  |
| 1,584,902    | Summers  | May 18, 1926   |
| 1,880,046    | Richter  | Sept. 27, 1932 |
| 1,883,478    | Bassett  | Oct. 18, 1932  |
| 1,924,815    | Skolnik  | Aug. 29, 1933  |
| 2,030,383    | Luth     | Feb. 11, 1936  |
| 10 2,030,384 | Luth     | Feb. 11, 1936  |
| 2,031,827    | Fiske    | Feb. 25, 1936  |
| 2,056,185    | Greene   | Oct. 6, 1936   |
| 2,074,473    | Jayme    | Mar. 23, 1937  |
| 2,219,432    | Scheller | Oct. 29, 1940  |

15 FOREIGN PATENTS

| Number     | Country       | Date          |
|------------|---------------|---------------|
| 417,035    | France        | June 11, 1910 |
| 358,144    | Germany       | Sept. 6, 1922 |
| 20 438,403 | Great Britain | Nov. 15, 1935 |
| 208,192    | Switzerland   | April 1, 1940 |

OTHER REFERENCES

- 25 Ser. No. 237,302, Passow (A. P. C.), published May 4, 1943.
- 25 American Dyestuff Reporter, Jan. 28, 1935, pp. 40-47.
- 30 Industrial and Engineering Chemistry, vol. 29, pp. 584-590 (1937).
- 30 Journal of Physical Chemistry, vol. 44, pp. 535, 539, 542, 570, 571 (1940).
- 35 Manufacture of Pulp and Paper, publ. by McGraw-Hill Book Co., New York, 3d Ed., vol. IV, Sec. 7, pp. 19 and 20 (1938).
- 35 Paper Industry and Paper World, May 1942, pp. 150 and 151.
- 40 Pacific Pulp and Paper Industry, Sept. 1940, p. 91.
- 40 Reprint from Oil and Soap, vol. 12, Feb. 1935.
- 40 Technical Association Papers Series 25, p. 327 (1942).